

## 1

3,446,333

**TREATING AUSTENITIC STAINLESS STEELS**  
Harshad J. Bhatt, Pittsburgh, and Peter R. Swann,  
Monroeville, Pa., assignors to United States Steel  
Corporation, a corporation of Delaware  
No Drawing. Filed June 7, 1966, Ser. No. 555,685  
Int. Cl. C21c 1/30, 1/60, 7/14

U.S. Cl. 148—12.4

10 Claims

This invention relates to austenitic stainless steels. More particularly, the invention concerns improving the resistance of austenitic stainless steels to stress corrosion cracking.

All stainless steels are iron-chromium alloys and may be grouped into three classes—martensitic, ferritic and austenitic. Generally, austenitic stainless steels are alloys of iron, chromium and nickel, with or without other elements. There are also austenitic stainless steels in which nickel is partially or wholly replaced by manganese and nitrogen.

Austenitic stainless steels have had wide-spread use as construction materials in nuclear reactors and in the chemical industry. However, it has been found that under certain adverse conditions such as exposure to chloride environments, austenitic stainless steels are susceptible to stress corrosion cracking. Because of the hazards associated with the failure of critical components in nuclear reactors as well as the expense involved in replacing components that have failed in the chemical industry, austenitic stainless steels with improved resistance to stress corrosion cracking are in demand.

The present invention concerns improving the resistance of austenitic stainless steels, with or without nickel, to stress corrosion cracking without sacrificing physical properties.

According to the invention, several different methods are provided for increasing the resistance to stress corrosion. Among the austenitic stainless steels with which the invention may be practiced are three of the most common types having AISI designations 301, 304 or 304L, 308 or 309, 310, and also partially or wholly nickel-free austenitic stainless steels. The first types of steel contain about 18% chromium, 8% nickel. The second type contains about 20% to 24% chromium, 12% nickel, and the third contains about 25% chromium, 20% nickel. Austenitic stainless steels in which nickel is partially replaced by manganese and nitrogen (AISI Type 201 and 202 stainless steels) contain about 18% chromium, 4% nickel, 7.5% manganese and 0.25% nitrogen. Nickel-free austenitic stainless steels contain about 18% chromium, 15% manganese and 0.50% nitrogen. Each of these steels may also contain small amounts of certain other elements added to enhance various properties or to immunize the steels against the action of certain harmful impurities and, in that event, are referred to by other AISI designations. Thus, the invention is applicable to related types of austenitic stainless steels as well as those referred to above.

The several processes within the purview of the invention are as follows:

(1) Low-temperature hot working of austenitic stainless steel followed by annealing at low optimum temperatures.

(2) Cold working either conventionally hot worked austenitic stainless steel or low-temperature hot worked steel followed by annealing at low optimum temperatures.

(3) Low temperature hot working followed by (with or without intermediate annealing) cold working and then conventional annealing of austenitic stainless steel.

(4) Conventional annealing of austenitic stainless steel followed by refrigeration at low temperatures to obtain

## 2

martensite and annealing to revert martensite to austenite; and

(5) Conventional annealing of austenitic stainless steel, cold working to obtain martensite, heating and annealing to revert martensite to austenite, refrigeration at a low temperature to obtain martensite and re-annealing to revert martensite to austenite.

The improvement in resistance to stress corrosion cracking obtained by practicing each of the above methods varies to some extent, but in every case represents at least 10-fold improvement. In some cases, the improvement may be as much as a 100-fold increase in the resistance to stress corrosion cracking.

Each of the several methods described above has some particular advantage which may affect its selection over the others in various situations. Method I is useful when high mechanical properties as well as high stress corrosion resistance is desired. Method II has the advantage that no special control of hot rolling is needed. Method III enables the use of conventional mill facilities and mill practices with optimum stress corrosion resistance obtained by use of the low-temperature finishing operation. Methods IV and V are practiced on metastable austenitic stainless steels and have the advantage that stress corrosion resistance can be obtained on steel products in an extremely deformed condition.

The methods referred to above will be individually described below. For comparison, conventional ingots of austenitic stainless steel were heated to hot working temperatures between 2100° F. and 2400° F., depending on composition, and then forged and/or hot rolled to semi-finished mill products such as blooms, billets and slabs. After conditioning, the semi-finished products are reheated and then hot rolled to finished mill products. The blooms or billets are customarily hot rolled to bars and rods, and the slabs are processed in a hot strip mill for the production of sheets or plates. The finished mill products are then annealed at a temperature between about 1900° F. and 2100° F. (usually at about 2000° F.) and rapidly cooled. Finishing operations, such as conditioning and cold reduction, are then performed.

## Method I

Contrary to the well-established practice, described above, we have discovered a marked improvement in resistance of austenitic stainless steels to stress corrosion cracking may be effected by lowering the conventional hot rolling finishing temperature and subsequent annealing temperatures. Moreover, the improvement obtained is achieved without sacrificing any of the critical mechanical properties such as formability and strength. In fact, it has been found that the yield strength is critically improved over those obtained with conventional processing. These advantageous results are obtained by hot working austenitic stainless steel ingots to a finishing temperature in the range of from about 1200° F. to about 1800° F., preferably about 1200° F. to about 1700° F., and subsequently annealing at temperatures between 1000° F. and 1600° F. followed by quenching. By "hot working" to the desirable "low finishing temperature" is meant that the hot working step is performed so that the last deformation is completed within the desired temperature range. Ordinarily, ingots are heated to starting temperatures higher than the finishing temperatures and cool during hot working. In the conventional practice, the hot rolled finishing temperature is above 1800° F.

As an illustration of the improved results obtained by practicing this method in accordance with the invention, two steels of AISI Type 304 and 304L were processed having the composition described in Table I.

TABLE I

| Steel         | Composition, percent |       |      |      |      |       |       |      |       |      |
|---------------|----------------------|-------|------|------|------|-------|-------|------|-------|------|
|               | C                    | N     | Ni   | Cr   | Mn   | P     | S     | Si   | Cu    | Mo   |
| Type 304L---- | 0.020                | 0.024 | 10.7 | 18.3 | 1.28 | 0.019 | 0.021 | 0.66 | 0.054 | 0.15 |
| Type 304----  | 0.038                | 0.025 | 9.65 | 18.3 | 1.31 | 0.022 | 0.016 | 0.43 | 0.035 | 0.23 |

The steel specimens were 1-inch thick plates which were hot rolled to 0.50-inch thickness in five passes of 0.1-inch reduction each. Both steels were rolled with a starting temperature of 2250° F. The finishing temperature for the Type 304L was 1600° F. and for the Type 304 was 1405° F. Other specimen blanks (0.5 x 0.5 x 3.0-inches) were cut from the hot rolled plates and tension-type specimens (0.252-inch diameter) were made from the blanks. The Type 304 and 304L specimens were annealed at 1200° F. and 1400° F., respectively, for 1 hour followed by quenching in ice water. The mechanical properties resulting from above treatments are shown in Table II. Comparison of processing by conventional practice is also shown in Table II. As is seen, the steels processed according to our invention show greatly increased yield strengths with other mechanical properties being substantially unchanged.

304 stainless steel cracked in an average of only 5 hours at a stress level of 22,500 p.s.i., whereas the same steel processed according to the invention lasted for an average of 255 hours before failure even when tested at the higher stress level of 41,000 p.s.i.

#### Method II

Conventionally, after hot rolling and mill annealing, austenitic stainless steels are conditioned and further reduced in thickness by a cold reduction process followed by annealing at about 2000° F. and rapid cooling. We have found, contrary to the well-established practice, that a marked improvement with respect to resistance of austenitic stainless steels to stress corrosion cracking may be effected by annealing the cold worked steels at lower than normal temperatures. Conventional annealing is performed at temperatures between 1900° F. and 2100° F.

TABLE II

| Steel         | Yield strength, p.s.i. |             | Tensile strength, p.s.i. |             | Reduction in area, percent |             |
|---------------|------------------------|-------------|--------------------------|-------------|----------------------------|-------------|
|               | Conv. proc.            | Impr. proc. | Conv. proc.              | Impr. proc. | Conv. proc.                | Impr. proc. |
| Type 304L---- | 34,000                 | 51,000      | 82,000                   | 87,000      | 80.0                       | 78.0        |
| Type 304----  | 30,000                 | 55,000      | 85,000                   | 90,000      | 81.0                       | 76.0        |

The superiority of the steels processed according to this method of the invention with respect to resistance to stress corrosion cracking is shown in Table III where this property is compared with that of austenitic steels of the same composition processed according to conventional practice. The steels are tested for stress corrosion properties in the customary manner by exposure to boiling magnesium chloride, a common testing medium, at a stress level of 75% of the actual yield strength of the test specimen.

35 To illustrate the results obtained with this method of the invention, two 300-pound ingots of the composition described in Table IV were heated to a hot working temperature of 2150° F. The ingots were hot rolled into 0.5-inch thick plate to a conventional finishing temperature of between 1800° F. and 1900° F. and subsequently 40 cooled in air. Specimen blanks (0.5 x 0.5 x 3.0-inches) were cut from the plates and were annealed at 1950° F. for 45 minutes followed by quenching in water. From the annealed blanks, tension-type specimens (0.252-inch diameter) were then machined. Some of these specimens were cold worked by elongating them about 30%, after which the specimens were annealed at 1400° F. for 1 hour followed by quenching in ice water. Mechanical properties, with or without the annealing treatment, are described in Table V. It can be noted that the steels 45 processed according to the invention show higher yield and tensile strengths than those processed according to the conventional practice.

TABLE III

| Steel         | Method of processing | Stress level, p.s.i. | Average <sup>1</sup> time to failure, hours | 45 |
|---------------|----------------------|----------------------|---------------------------------------------|----|
|               |                      |                      |                                             |    |
| Type 304L---- | Conventional         | 25,600               | 10                                          |    |
|               | Improved             | 38,300               | 2458                                        |    |
| Type 304----  | Conventional         | 22,500               | 5                                           | 50 |
|               | Improved             | 41,000               | 255                                         |    |

<sup>1</sup> Average of three specimens.

<sup>2</sup> Average of two specimens.

| Steel  | Composition, percent |       |      |      |      |       |       |      |  |
|--------|----------------------|-------|------|------|------|-------|-------|------|--|
|        | C                    | N     | Ni   | Cr   | Mn   | P     | S     | Si   |  |
| A----- | 0.014                | 0.007 | 12.7 | 17.6 | 1.49 | 0.023 | 0.019 | 0.50 |  |
| B----- | 0.064                | 0.110 | 17.9 | 18.1 | 1.60 | 0.026 | 0.013 | 0.56 |  |

| Steel  | Yield strength, p.s.i. |             | Tensile strength, p.s.i. |             | Reduction in area, percent |             |
|--------|------------------------|-------------|--------------------------|-------------|----------------------------|-------------|
|        | Conv. proc.            | Impr. proc. | Conv. proc.              | Impr. proc. | Conv. proc.                | Impr. proc. |
| A----- | 28,000                 | 31,000      | 72,000                   | 80,000      | 78.4                       | 77.7        |
| B----- | 39,000                 | 79,000      | 88,000                   | 107,000     | 75.6                       | 61.1        |

The conventionally processed Type 304L cracked in this solution in an average of 10 hours at a stress level of 25,600 p.s.i. In contrast, steel processed according to the invention lasted for an average of 458 hours before cracking even when tested at the higher stress level of 38,300 p.s.i. Similarly, conventionally processed Type

75 The superiority of the steels processed according to the invention with respect to their resistance to stress corrosion cracking are shown in Table VI. Conventionally processed steel A cracked in a boiling magnesium chloride solution within an average of 39 hours at a stress level of 21,000 p.s.i. The same steel processed according

to the invention did not fail with an average of 555 hours when tested at a stress level of 23,000 p.s.i. under identical conditions. The steel B cracked in a boiling magnesium chloride solution within an average of 67 hours at a stress level of 29,000 p.s.i., whereas the same steel processed according to the invention did not fail within 5

The superiority of the steel processed according to our invention with respect to its resistance to stress corrosion cracking is shown in Table VIII, wherein the conventionally processed Type 304L stainless steel is compared with a similar steel processed in accordance with the invention.

TABLE VIII

| Steel                | Method of processing | Treatment                                                                                                                     | Average time to failure, hours |
|----------------------|----------------------|-------------------------------------------------------------------------------------------------------------------------------|--------------------------------|
| C                    | Improved             | Hot rolled; cold-reduced (50%); annealed at 2,000° F., 1 minute; air cooled                                                   | 1,000                          |
| C                    | do                   | Hot rolled; annealed at 1,950° F., 15 minutes; W.Q.; cold reduced (50%); annealed at 2,000° F., 1 min. or 5 min.; air cooled. | 1750                           |
| Commercial Type 304L | Conventional         | Mill annealed                                                                                                                 | 2                              |

<sup>1</sup> No failure at indicated times.

515 hours, although it was tested at a stress level more than twice (59,000 p.s.i.) that used for the conventionally processed specimens.

TABLE VI

| Steel | Method of processing | Stress level, p.s.i. | Average <sup>1</sup> time to failure, hours |
|-------|----------------------|----------------------|---------------------------------------------|
| A     | Conventional         | 21,000               | 39                                          |
| A     | Improved             | 23,000               | 2 555                                       |
| B     | Conventional         | 29,000               | 67                                          |
| B     | Improved             | 59,000               | 2 515                                       |

<sup>1</sup> Average of four specimens.

<sup>2</sup> No failure at indicated times.

### Method III

The advantage of this method of the invention is that it can employ conventional annealing temperatures and special annealing practices need not be observed. This method comprises low temperature hot working followed by heavy cold reduction and subsequent annealing at conventional temperatures, or hot working at low temperature followed by annealing and cold reduction with a subsequent final conventional anneal.

To illustrate the improved properties of steel processed in accordance with this method of the invention, a 300-pound vacuum melted ingot of a steel of composition C, shown in Table VII, was heated to 2150° F. for 1½ hours and then hot rolled to 0.755-inch thick plate in eight passes to a finishing temperature of about 1675° F. prior to air cooling. The plate was then further hot rolled from 0.755-inch plate to 0.117-inch thick sheet. The starting temperature as well as the number of hot rolling passes were the same as in the first hot rolling operation, but the finishing temperature was between 1500° F. and 1600° F. After air cooling, the sheet was then cold reduced to 0.050-inch thick, annealed at 2000° F. for 1 minute in a salt bath, and cooled in air. The chemical compositions of this steel as well as the commercial Type 304L are given in Table VII.

25 The conventionally processed steel Type 304L cracked in the boiling magnesium chloride solution within an average of 2 hours, whereas the steel processed in accordance with the invention did not crack within 1000 hours in the same test. Also, introducing an intermediate annealing treatment between the hot working and the cold working operations does not eliminate the improvement obtained by the application of this method.

### Method IV

30 This method and Method V described below are particularly well suited to metastable austenitic stainless steels. Typical of these steels are AISI Types 301, 304 and 304L. Because of the metastability, a special practice is observed to increase the martensite development for availability in reverting to austenite.

35 Contrary to the well-established conventional practices, it has been discovered that in these metastable steels, resistance to stress corrosion cracking may be achieved by refrigerating annealed austenitic stainless steels at very low temperatures to obtain a substantially martensitic structure, and then reverting to martensite formed to austenite by annealing at conventional temperatures, usually about 2000° F. or at a lower temperature just above the temperature at which martensite transforms to austenite.

40 The superior properties of the product produced in accordance with this method of the invention is shown by the following example. Steels D and E of chemical composition shown in Table IX, which are similar to AISI Type 301 stainless steel, were prepared in 300-pound vacuum, induction-melted ingots. The ingot of steel composition D was hot rolled to 0.50-inch thick plate. Some of these hot rolled plates were annealed at 1950° F. for about 45 minutes and then quenched in water. Specimen blanks 0.5 x 0.5 x 0.3-inches were cut from the hot rolled plates as well as from the hot rolled plus annealed plates and 0.252-inch diameter tension specimens were made from the blanks. Some were given the

TABLE VII

| Steel     | Composition, percent |       |     |      |      |       |       |      |
|-----------|----------------------|-------|-----|------|------|-------|-------|------|
|           | C                    | N     | Ni  | Cr   | Mn   | P     | S     | Si   |
| C         | 0.019                | 0.035 | 7.9 | 17.9 | 1.50 | 0.027 | 0.015 | 0.53 |
| Type 304L | 0.02                 | 0.026 | 9.4 | 19.6 | 1.28 | 0.022 | 0.017 | 0.61 |

70 Olsen cup specimens were used to determine the effect of deformation on the stress corrosion properties of the sheet. This involves indenting a 3¾ x 4-inch sheet with a ½-inch diameter ball to 75% of the extension required to fracture the sheet. The Olsen cup specimens were then exposed to a boiling 42% magnesium chloride solution.

75 double phase transformation treatment described previously. In this method, the hot rolled steels were annealed at about 1950° F. or a lower temperature of 1400° F., and the annealed specimens were refrigerated in liquid nitrogen at -320° F. to obtain martensite. The martensite was then reverted to austenite by heat treating at 1950° F. or 1400° F. As may be seen from

Table X, this cycle was in some experiments repeated twice. It should be understood however that the cycle may be repeated as many times as required to achieve the desired properties.

TABLE IX

| Steel  | Chemical composition, percent |       |     |      |      |       |       |      |
|--------|-------------------------------|-------|-----|------|------|-------|-------|------|
|        | C                             | N     | Ni  | Cr   | Mn   | P     | S     | Si   |
| D----- | 0.044                         | 0.005 | 7.9 | 17.6 | 1.51 | 0.025 | 0.017 | 0.49 |
| E----- | 0.019                         | 0.035 | 7.9 | 17.6 | 1.50 | 0.027 | 0.015 | 0.53 |

The superior resistance to stress corrosion cracking of the specimens processed according to this method of the invention is shown in Table X. In this table, a comparison of the properties of specimens made from the same steel but processed by conventional practice and with the properties of specimens processed in accordance with this method of the invention are shown. After heat treating, the specimens were prestrained 10-30%, stressed to 75 or 100% of the load required to obtain the prestrain, and exposed to a boiling 42% magnesium chloride solution. The specific heat treatments, amount of prestrain, and the stress corrosion results are given in Table X.

TABLE X

| Method of processing | Amount of prestrain, percent      | Stress level                  |                        | Time to failure, hr. |             |
|----------------------|-----------------------------------|-------------------------------|------------------------|----------------------|-------------|
|                      |                                   | Percent of load for prestrain | Pounds per square inch | 1                    | 2           |
| Conventional -----   | HR+A (1,950° F.)                  | 10                            | 75                     | 42,800               | 4 -----     |
| Improved-----        | HR+A (1,950° F.)+R+A (2,000° F.)  | 10                            | 75                     | 51,300               | 1 528 ----- |
| Conventional -----   | HR+A (1,950° F.)                  | 15                            | 75                     | 63,700               | 5 -----     |
| Improved-----        | HR+A (1,950° F.)+R+A (2,000° F.)  | 15                            | 75                     | 52,900               | 160 -----   |
| Do-----              | HR+A (1,400° F.)+R+A (1,400° F.)+ | 15                            | 100                    | 127,100              | 1 760 ----- |
|                      | R+A (1,400° F.).                  |                               |                        |                      |             |
| Conventional -----   | HR+A (1,950° F.)                  | 20                            | 75                     | 69,300               | 3 -----     |
| Improved-----        | HR+A (1,950° F.)+R+A (2,000° F.)  | 20                            | 75                     | 83,600               | 8 -----     |
| Conventional -----   | HR+A (1,950° F.)                  | 30                            | 75                     | 100,000              | 4 -----     |
| Improved-----        | HR+A (1,400° F.)+R+A (1,400° F.)+ | 30                            | 75                     | 119,600              | 1 600 ----- |
|                      | R+A (1,400° F.).                  |                               |                        |                      |             |

<sup>1</sup> No failure at indicated times.  
HR—Hot rolled; A—Annealed; R—Refrigerated in liquid nitrogen (-320° F.).

TABLE XI

| Method of processing | Amount of prestrain, percent                                         | Stress level                  |                        | Time to failure for one specimen, hr. |
|----------------------|----------------------------------------------------------------------|-------------------------------|------------------------|---------------------------------------|
|                      |                                                                      | Percent of load for prestrain | Pounds per square inch |                                       |
| Conventional -----   | HR+A (1,950° F.)                                                     | 5                             | 75                     | 36,500                                |
| Improved-----        | HR+A (1,200° F.)+R+A (1,200° F.)+R+A (1,200° F.)                     | 5                             | 75                     | 54,000 118                            |
| Do-----              | HR+D (20%)+A (1,200° F.)+R+A (1,200° F.)+R+A (1,200° F.)             | 5                             | 75                     | 66,200 218                            |
| Do-----              | HR+D (20%) at -320° F.+A (1,200° F.)+R+A (1,200° F.)+R+A (1,200° F.) | 5                             | 75                     | 92,200 1 571                          |
| Do-----              | HR+D (20%) at -320° F.+R repeated four times                         | 5                             | 75                     | 29,800 6                              |
| Do-----              | HR+A (2,000° F.)+R repeated four times                               | 5                             | 75                     | 55,900 195                            |
| Do-----              | HR+A (1,200° F.)+R repeated four times                               | 5                             | 75                     | 128,300 1 644                         |
| Do-----              | HR+D (20%) at -320° F.+A (1,200° F.)+R+A (1,200° F.)                 | 17                            | 75                     |                                       |

<sup>1</sup> No failure at indicated times.  
HR—Hot rolled; A—Annealed; R—Refrigerated in liquid nitrogen (-320° F.); D—Cold worked by elongation.

As can be seen, at least a 100-fold improvement in stress corrosion resistance was obtained in the specimens processed in accordance with the invention. The results also show that the degree of improvement depends on the annealing temperature as well as the reversion temperature used. For example, as shown in Table XI, when hot rolled steel is annealed at 2000° F. and refrigerated with the cycle being repeated four times before final annealing, the specimen failed in 6 hours. In contrast, when the same hot rolled steel was annealed and refrigerated with the cycle being repeated four times before final annealing at 1200° F., the specimen failed in 195 hours. It should further be noted that this improvement is achieved even though this specimen was tested at almost double the stress level of the other specimen. The optimum temperature for annealing of the hot rolled specimens as well as the reversion of martensite to

75 substantially below room temperature, e.g. -75° F. or lower. Steels with higher  $M_s$  temperatures, e.g. -30° F., can be treated successfully according to Method IV.

In this method according to the invention, hot rolled steels are annealed and then cold reduced either at room temperature or preferably at a temperature as low as that of liquid nitrogen (-320° F.). In this manner, the austenite can be substantially transformed to martensite. Martensite is then reverted to austenite by heat treating at least at the  $A_f$  temperature, i.e. the temperature at which martensite is reverted to austenite. This is indicated by a lack of any magnetic activity, as can be determined by a hand magnet. Following reversion to austenite, Method IV is then applied and the steel is refrigerated at very low temperature to obtain a substantially martensitic structure and then exposed to elevated temperatures to revert martensite to austenite.

austenite has been found to be at about 1200° F. for these representative compositions. The minimum temperature for reversion does vary to some degree with the composition of the steel and a substantial grain can be

As an example of this method according to the invention, steels of composition E (see Table IX) were prepared in 300-pound vacuum induction melted ingots and hot rolled to 0.5-inch thick plates. Some of these plates were annealed at 1950° F. for about 45 minutes and quenched in water. Specimen blanks 0.5 x 0.5 x 3.0-inches were cut from hot rolled plus annealed plates and tension specimens were made from the blanks. Some specimens were given the double phase transformation described above, i.e. refrigeration followed by annealing above the  $A_f$  temperature, preferably at about 1200° F.

The superior resistance to stress corrosion cracking of the steel processed in accordance with this method of the invention is shown in Table XI above, wherein these results are compared with those obtained for specimens made from the same steel but processed by the conventional practice. After heat treating, the specimens were restrained, stressed to 75% and exposed to a boiling 42% magnesium chloride solution. The specific heat treatments, amounts of prestrain and stress level and stress corrosion results are given in Table XI. More than a 100-fold improvement was obtained on the specimens processed according to this method of the invention.

It is apparent from the above that various changes may be made without departing from the invention. Accordingly, the scope of the invention should be limited only by the appended claims.

We claim:

1. A method of improving the resistance of austenitic stainless steels to stress corrosion cracking which comprises hot working said steel to a finishing temperature in the range of from about 1200° F. to about 1800° F., low temperature annealing in the range of from about 1000° F. to about 1600° F. and thereafter quenching.

2. A method according to claim 1 wherein said low temperature annealing is performed at about 1200° F.

3. A method according to claim 1 wherein said low temperature annealing is performed at about 1400° F.

4. A method of improving the resistance of austenitic stainless steels to stress corrosion cracking which comprises cold working austenitic stainless steel which has been hot worked, annealing said cold worked steel in the

temperature range of from about 1200° F. to about 1800° F. and thereafter quenching.

5. A method of improving the resistance of austenitic stainless steel to stress corrosion cracking which comprises hot working said steel to a finishing temperature in the range of from about 1200° F. to about 1800° F., cold working said steel and annealing said cold worked steel at temperature in the range of from about 1900° F. to about 2100° F.

10 6. A method according to claim 5 wherein said steel is hot worked to a finishing temperature in the range of from about 1200° F. to about 1700° F.

15 7. A method of improving the resistance of metastable austenitic stainless steel to stress corrosion cracking, which comprises annealing said steel, refrigerating said steel at a low temperature sufficient to obtain a substantially martensitic structure and annealing at temperature in the range of from about 1200° F. to about 2000° F. to revert martensite to austenite.

20 8. A method according to claim 7 wherein said steel is refrigerated and annealed more than once.

25 9. A method of improving the resistance of metastable austenitic stainless steel to stress corrosion cracking which comprises annealing said steel, cold working said steel until the steel becomes strongly magnetic, heating said steel to revert martensite to austenite and annealing same, refrigerating said steel at a low temperature sufficient to obtain a substantially martensitic structure and annealing at a temperature above the  $A_f$  temperature to revert martensite to austenite.

10. A method according to claim 9 wherein said annealing above the  $A_f$  temperature is performed at about 1200° F.

#### References Cited

#### UNITED STATES PATENTS

|           |         |           |       |          |
|-----------|---------|-----------|-------|----------|
| 2,820,708 | 1/1958  | Waxweiler | ----- | 148—12.3 |
| 2,363,736 | 11/1944 | Lynn      | ----- | 148—12.4 |
| 2,266,952 | 12/1941 | Bloom     | ----- | 148—12.4 |

L. DEWAYNE RUTLEDGE, Primary Examiner.

W. W. STALLARD, Assistant Examiner.